

1,213,555

## UNITED STATES PATENT OFFICE.

ROBERT FULTON TOMPKINS, OF NEW YORK, N. Y., ASSIGNOR TO THE BINDER COMPANY,  
A CORPORATION OF NEW JERSEY.

## ROADWAY COMPOSITION.

1,213,555.

Specification of Letters Patent. Patented Jan. 23, 1917.

No Drawing.

Application filed August 15, 1913. Serial No. 784,885.

106 - 287

*To all whom it may concern:*

Be it known that I, ROBERT FULTON TOMPKINS, citizen of the United States, residing at New York city, in the county of 5 New York and State of New York, have invented certain new and useful Improvements in Roadway Compositions, of which the following is a specification.

This invention relates to roads or roadways and process of constructing the same and has for its object the formation of compounds or substances with or from constituents of a road body, base, or dressing which are of cementitious nature, by exposing the 15 associated materials to the action of carbon-containing acids, such as tannic, resinic, aliphatic, etc. or substances capable of forming, yielding, producing or delivering such acid in the presence of the material to be 20 bonded or cemented.

As an example of a road constructed in accordance with the present invention, a road or roadway of the macadam or similar type associated with ingredients and constructed in accordance with the present invention, will be taken as an illustration.

The macadam type of road or roadway is formed of a vehicle carrier or matrix containing substances such as compounds of 30 iron, calcium, magnesium and the like, capable of forming water resistant compounds with carbon-containing acids, such as tannic acid, capable of uniting with the metal base of such compounds and uniting the same in 35 a cementitious manner. The said road or roadway is provided with a top dressing of similar material associated with the usual finer grades of mineral filler, the ingredients of the top dressing being caused to cohere 40 and adhere by means of the metal tannates directly or indirectly formed when associated therewith.

A construction of this character thus provides a superior cementing agent of non-volatile nature, having sufficient natural moisture retaining properties, while of inherent water-repellent nature, to prevent drying out while causing the solid particles of the roadway or roadbed to cohere or 45 adhere in a flexible, resilient and elastic manner.

In constructing the roadbed, the ordinary ingredients, such as broken stone, sand, gravel and the like, are mixed after the or-

dinary well known fashion, and this road body is mixed with an organic or carbon-containing acid or substance containing the same, such as tannic acid or tannic acid associated with such vehicles as are ordinarily present in the tanning extracts of barks or woods, in proportion of one of the concentrated liquor containing approximately 25 per cent. of tannic acid or substances capable of yielding the same, to three of water by volume. The road construction material is mixed with this tannic acid-containing or yielding liquor, in sufficient amounts to moisten the particles of contacting substance, and then the whole mixed with suitable mineral cementitious or other 70 uniting or binding substances, such, for instance, as cement, forming concrete, and the composition spread, rolled, tamped or otherwise placed in proper position or location whereby it will become set or fixed in composite form as a road-body.

The road bed, when it has been properly provided as aforesaid is spread with a top dressing of granulated or finely divided material, associated with tannic acid or 80 tannic acid producing, yielding or delivering substances, such as the extract of barks and woods, and more particularly such materials as extract of chestnut wood and the like which are adaptable for the tannage of 85 skins in the production of leather. This dressing is then rolled in and upon the roadway forming a compact dressing of more or less water-repellent nature, but of sufficient water-absorbent character to retain the moisture and prevent drying out and dusting of the composition.

Instead of a cement concrete base, containing the binder as aforesaid, having a direct top dressing of the character described, the materials of the road bed may be primarily dressed with an asphalt composition upon which a top dressing or finish is placed in communication with the asphalt layer, comprising sufficiently granulated or 100 comminuted frictional substances, such as sand, associated with tannic acid or tannic acid-forming, yielding, delivering or bearing substances, in such a manner that the frictional substances are anchored to, cemented by, or united with a surface of the asphalt coating.

Some of the advantages of a road of this

character over roads constructed hitherto, resides in the fact that the comminuted particles of the road produced by wear and tear during use by tires of vehicles and the like, are held together by the natural binding, or cementing character of the metal tannate produced and present and prevented largely from being converted into dust by circulation in currents of air actuated by the movement of vehicles. The moisture occluded or held by the metal tannates being displaced under pressure of the vehicle weight upon it, catches and secures any associated fine material in juxtaposition thereto, and holds the same to the contacting material containing the metal tannates while under pressure, and thereafter when the elastic tannates recover or resume their original volume by expansion.

The action of heat on a road bed or road of the character of the present invention does not have the effect of destroying the cohering and adhering properties of the binding or cementing tannate or non-volatile metal tannic acid compound retaining moisture, as is the case where oils are employed which are of more or less dry or volatile character.

Where oil alone is used to cause the coherence or adherence of particles in a road or road dressing, it is not only lost by evaporation and drying out, but it likewise reduces the gravity of the fine contacting particles of the road dressing so that water, from rain or other source, causes it to float and be carried off. Oil also produces an injurious and disintegrating effect upon vehicle tires and greases and destroys the appearance of varnish and other finish upon vehicles, exerts a deleterious action on metal, wood and leather, as well as creating a greasy, dusty atmosphere, injurious to the eyes and clothes and which also settles in houses upon furniture and other contents in the vicinity and contaminates water upon which it falls, such as contained in reservoirs and the like, and also forms a sticky contamination on clothes, which is hard to remove, all of which disadvantages are obviated by the employment of metal carbon-containing acid, salts or compound employed as binding or cementing agents such as metal tannates, which metal tannates or compounds of carbon-containing acids before noted are of water-repellent but water-retaining character, and form, in conjunction with other materials, when cementing the same, as a mineral road dressing, a substance of greater gravity or increasing gravity with relation to water, than oil, so that it is not so readily washed away, and at the same time maintains the road dressing in a naturally and progressively moist condition by taking up or absorbing moisture from the atmosphere automatically, to compensate for

the moisture dislodged or dissipated by evaporation through the action of heat, such as the sun, etc., due to the binding or cementing constituent's inherent properties, of hygroscopic nature.

Asphalt roads or roadways dressed with frictional substances, such as sand, bonded or united with metal carbon-containing compounds or salts such as metal tannate of hygroscopic nature, holds down the dressing against the flow of water over the impermeable asphalt containing surface, and the dressing thus retained or anchored to the asphalt will largely enhance the friction of the road surface under pressure, or attrition and retard the slipping of horses' shoes and the skidding of vehicle tires, the slipping and skidding of which presents one of the greatest difficulties and objections to the employment of asphalt as a top dressing per se, and it also provides a means for anchoring sheeted particles of ice, which may form on the road bed, to the surface of the asphalt, thereby increasing the utility of asphalt roads and preventing this other serious objection to their employment. The composite coating or dressing of mineral substances bonded together by metal carbon-containing acid salts or compounds, also forms a gravity blanket comprising cohering and adhering particles when employed in conjunction with the roadbed of existing roads, railroads or other viaducts for vehicles or other purposes, whereby the cemented aggregated material is collectively retained against currents of air and the road bed protected against water and currents thereof removing the surface. This material spread upon such roads as asphalt roads not only provides a superior surface of frictional nature, but also protects the asphalt surface against wear and loss of volatile constituents, which is often occasioned by the action of the heat of the sun, thus prolonging the life and utility of such treated asphalt-containing roads.

The average composition of chestnut wood extract referred to as an applicable species or constituent to be employed as a vehicle or carrier, or deliverer of tannic acid to constituents of a road or road dressing, or substances to be employed with relation thereto, is as follows: soluble tannin 25.22%, non-tannins 15.85, insolubles 0.35, soluble solids 41.07, total solids 41.42, moisture 58.58. This composition being preferably diluted when applied to the surface of a finished road with water in proportion of one of the compositions to three of the water, and the diluted composition applied by means of sprinkling so that as the substance is absorbed into the road dressing, surface or road bed, the acid content reacts or combines with the metal base of the compounds present, such as compounds of iron,

calcium, magnesium and the like, and forms therewith a chemically cemented binder of water-repellent and water-retaining character.

5 The carbon-containing acid employed may be of individual character or associated with, combined or carried in suitable vehicle so long as it is delivered directly or indirectly to the metal of the metal-containing 10 substances of the road or roadway existing as such, or materials to be employed in its construction.

Instead of mixing the tannic acid or tannic-acid bearing or delivering substance 15 directly with the constituents of the road construction during the road building, it may be applied to a road or roadway after the same is constructed, by sprinkling a sufficiently fluid solution upon the road and allowing it to soak in, and preferably rolling the same thereafter to form a compact top dressing, and this mixture, when sprinkled upon or otherwise applied to the road surface, and allowed to soak in is preferably 20 subjected to a second sprinkling or wetting by slightly more dense liquor consisting of approximately one part of the concentrated material, such as the chestnut wood extract of the composition before noted, to two of 25 water, the interval of time between the two applications being sufficient to allow the first coat to be absorbed and combined in such a manner as to act both as a cementing agent and as a leader or path for the more dense liquor to be absorbed, and for the purpose of 30 rolling and setting to be accomplished. The metal tannates, such as tannates of iron aluminium, calcium, magnesium and the like, being of substantially insoluble nature, combine or include the property of absorbing 35 moisture without disintegration, and are reaching out for or absorbing moisture from the atmosphere under all favorable conditions and maintaining the ingredients bonded by them in a sufficiently moist condition 40 to be resilient and elastic, without enhancing the binding properties or injuring the cemented character of the material.

The metal compounds or salts formed by 45 the combination of carbon-containing acids such as tannic acids, provide a superior bonding vehicle or material for the constituents of road bodies or dressings, and it is here intended to include all such metal carbon-containing acid compounds or salts of 50 substantially insoluble nature, but of more or less hygroscopic character, such as the metal salts or compounds of resin acids and others of waxy, gummy sticky or fatty nature, of which tannic acid is a species.

The tannic acid employed may be applied 55 as free acid either alone or associated with other vehicles, substances or fillers, or it may be derived from substances capable of yielding same by decomposition or disas-

sociation either by action of the road bed constituents, or substances intended therefor, or other means at or prior to its association. Some of the materials from which tannic acid may be derived may be noted as the glucosids which are ethereal salts or esters of tannic acid, or substances containing the same otherwise united, such as the materials known as sulfite pulp waste, which carries aldehydes and ketones capable of forming and delivering tannic acid upon decomposition.

70 The tannates employed as binding agents may be also noted as exhibiting the additional property of being antiseptics and germicides so that dust associated with such material would not act as a disease-carrying medium.

75 It is sometimes found advisable to mix with substances of the character of the chestnut wood extract referred to, other substances carrying more solid matter or other fillers, such as a concentrated spent tan bark liquor which is now generally thrown away at the tanneries, or associating therewith 80 such substances as sulfite pulp waste or substances derived therefrom.

85 It will be noted that this invention is particularly directed to the metal carbon acid salts or compounds, such as tannic acid compounds or salts of metal in contra-distinction to and from the ethereal salts or esters of tannic acid and the like as described and claimed in a companion application, Serial Number, 784,884.

90 Another source of carbon-containing acid 100 may be noted as that which occurs during the oxidation of an aldehyde so that this invention includes the direct formation of such acids by associating materials capable of forming the same, such as an aldehyde subjected to oxidation in the presence of substances capable of combining with the acid produced either directly or after such acid is formed, as well as the employment 105 of free acid *per se* or acid derived from other sources such compounds of organic or other nature capable of yielding or delivering the same upon chemical transformation, reaction, or dissociation.

110 Having now described my invention, what I claim as new and desire to secure by Letters Patent is:—

1. A road or roadway composition, comprising a road base and binding substance 115 including a water-insoluble metal compound of a carbon-acid of aromatic type.

2. A road or roadway composition comprising a road base, a filler, and a water-insoluble metal compound of a carbon-acid 120 of aromatic type.

3. A road or roadway composition comprising a road base, a filler, a dressing and a water-insoluble metal compound of a carbon-acid of aromatic type.

4. A road or roadway composition, comprising a road base and binding substance including a water-insoluble metal compound of tannic acid.
5. A road or roadway composition comprising a road base, a filler, and a water-insoluble metal compound of tannic acid.
6. A road or roadway composition comprising a road base, a filler, a dressing and a water-insoluble metal compound of tannic acid.
- 10 7. A road or roadway, comprising a road base and binding substance including a water-insoluble metal salt of a carbon-hydrogen acid of aromatic type.
- 15 8. A road or roadway composition comprising a road base, a filler, and a water-insoluble metal salt of a carbon-acid of aromatic type.
- 20 9. A road or roadway composition comprising a road base, a filler, a dressing and a water-insoluble metal salt of a carbon-acid of aromatic type.
- 25 10. A road or roadway composition, comprising a road base and binding substance, including a water-insoluble metal salt of tannic acid.
- 30 11. A road or roadway composition comprising a road base, a filler, and a water-insoluble metal salt of tannic acid.
12. A road or roadway composition comprising a road base, a filler, a dressing and a water-insoluble metal salt of tannic acid.
- 35 13. A road or roadway composition, comprising a road base and a binding substance including a water-insoluble metal tannate.
14. A road or roadway composition, comprising a road base, a filler, and a water-insoluble metal tannate.
15. A road or roadway composition comprising a road base, a filler, and a water-insoluble metal tannate.
16. A road or roadway composition comprising a road base, a filler, a dressing and a water-insoluble metal tannate.
17. A road or roadway composition comprising a road base, a filler, and iron tannate.
18. A road or roadway composition, comprising a road base, a filler, a dressing and iron tannate.
19. The combination in a road or roadway of a bonding substance comprising a metal compound of a carbon acid of aromatic type.
20. The combination in a road or roadway of a bonding substance comprising a water-insoluble metal compound of tannic acid.
21. The combination in a road or roadway of a bonding substance comprising a metal salt of a carbon acid of aromatic type.
22. The combination in a road or roadway of a bonding substance comprising a water-insoluble metal tannate.
23. The combination in a road or roadway of a bonding substance comprising iron tannate.
- In testimony whereof I affix my signature in presence of two witnesses.
- ROBERT FULTON TOMPKINS. [L. S.]
- Witnesses:
- Wm. J. JULIEN,  
RALPH E. HALLOCK.